

# UNITED STATES PATENT OFFICE.

JOSEPH WADE TUCKER, OF KISSIMMEE, FLORIDA, AND WILLIAM A. MCCOOL, OF BEAVER FALLS, PENNSYLVANIA.

## METHOD OF MAKING BRICKS AND THE LIKE.

1,220,293.

Specification of Letters Patent. Patented Mar. 27, 1917.

No Drawing.

Application filed November 20, 1916. Serial No. 132,326.

*To all whom it may concern:*

Be it known that we, JOSEPH WADE TUCKER and WILLIAM A. MCCOOL, citizens of the United States, residing, respectively, 5 at Kissimmee, in the county of Osceola and State of Florida, and Beaver Falls, in the county of Beaver and State of Pennsylvania, have invented certain new and useful Improvements in Methods of Making Bricks 10 and the like, of which the following is a specification.

This invention relates to a method or process for producing bricks, blocks or the like, for paving or other purposes, and has for 15 its object to provide bricks or blocks of low cost, which will afford a cushioning or noise and shock deadening traffic surface, which are sufficiently strong, durable and wear-resisting to perform their intended function 20 in an efficient manner, which are waterproof and durable, and which are unaffected by any degree of heat to which they are likely to be subjected, or by saline solutions, acids, or other chemical agencies, the last-named 25 characteristic making such bricks or blocks especially suitable for paving purposes in stables, shops, and other places in which such destructive agencies are frequently encountered.

30 The foregoing and other objects of the invention will best be understood from the following detailed description of the manner in which the same may be carried into effect.

35 In accordance with said invention the bricks, blocks or the like are composed of an aggregate comprising a comminuted, absorbent organic material treated with a suitable substance which impregnates the same, 40 and a binder which, under heavy pressure, unites said aggregate into a solid mass. Said absorbent material may be any non-resinous wood but preferably consists of comminuted cypress wood, either in 45 shredded form, produced from scrap, or as sawdust, this material having been found especially suitable for the purpose by reason of its cheapness in certain localities, its durability, and its substantial freedom from pitch, resin or other substances which might 50 interfere with its thorough impregnation. The substance with which said absorbent comminuted wood is impregnated, as also the binder by which it is united, are both

preferably derived from the heavy and 55 otherwise comparatively useless hydrocarbon residues produced in the refining of crude mineral oils having an asphalt base, said residue comprising a mixture of asphaltums of different melting points and being left after the extraction from the crude oil of the more volatile components, such as gasoline, naphtha, kerosene, etc. These residues are subjected to a fractional distillation (preferably at a temperature of 60 from 240° F. to 260° F.) by which the lighter components thereof are separated from the heavier, that is to say, the asphaltums of relatively low melting point are separated from those of relatively high 65 melting point. The comminuted wood is first soaked for a sufficient length of time (preferably from 15 to 20 minutes) in an excess of the lighter or low melting point asphaltums, to cause the wood particles to 70 be thoroughly impregnated with the thin or light asphaltum substance, which, of course, is in melted or liquid form. Said impregnated comminuted wood is thereafter thoroughly mixed with a sufficient quantity of 75 the heavier hydrocarbon material, or high point asphaltums, also in a melted condition, to be thoroughly coated therewith. Preferably only a sufficient quantity of the heavier asphaltum is employed to coat the aggregate completely and to bind the same firmly 80 together without excess. Suitable proportions have been found to be about 82 parts of the impregnated comminuted cypress wood to about 18 parts of the binder, although 85 these proportions are capable of considerable variation. The comminuted wood thus impregnated and thoroughly mixed with the binder, by any suitable means, is molded into blocks or bricks of suitable 90 shape and size and under a heavy pressure in a hydraulic or other suitable press of any well-known character.

A brick or block made as above described has been found admirably to fulfil all of the 95 conditions, and to possess all of the desirable qualities, heretofore referred to. In order to meet said conditions it is necessary that the comminuted wood be thoroughly impregnated with a material which will 100 render the same waterproof and that it be bound together by a material which will 105 afford the necessary strength and dura-

bility and which is not readily inflammable or injuriously affected by heat. Any hydrocarbon or other similar material capable of fulfilling the first-named conditions has 5 been found in practice to be too light to form a sufficiently strong binder to provide the necessary strength and durability. On the other hand, it has also been found in practice that any hydrocarbon heavy enough 10 to serve as a suitable binder is too heavy to penetrate the pores of the wood, but merely coats the surfaces of the particles of the aggregate and binds them together. In such case the wood particles are not properly impregnated and waterproofed by such 15 heavy binder.

In the bricks or blocks above described the lighter asphaltums serve effectually to impregnate and waterproof the comminuted 20 wood, while the heavier asphaltums serve as a highly efficient binder. Moreover, it is found that, when the impregnated comminuted wood is mixed with the binder and subjected to pressure, such lighter and 25 heavier asphaltums display a strong affinity for one another and recombine to form a more or less homogeneous compound which entirely permeates the aggregate and binds the same together; which is strong and durable; which is capable of resisting a heat 30 of 200° F., or more; and which is not affected by saline solutions, acids, or other destructive chemical agencies.

The terms "bricks" and "blocks" as herein 35 used are to be taken as broad and general in their meaning and to include paving or structural elements of any form or size suitable for the uses to which they are to be put, and capable of being manufactured 40 as above described.

The product of the method or process above described, is not herein claimed but forms the subject-matter of another application filed by us simultaneously herewith,

45 No. 132,325.

Having thus described our invention or

discovery we claim and desire to secure by Letters Patent:

1. The herein described method of making 50 bricks, blocks, or the like, which consists in impregnating a comminuted non-resinous wood with a relatively light hydrocarbon material and uniting the same into a solid 55 mass, under heavy pressure, by means of a relatively heavy hydrocarbon material.

2. The herein described method of making 60 bricks, blocks, or the like, which consists in impregnating comminuted cypress wood with a relatively light hydrocarbon material and uniting the same into a solid 65 mass, under heavy pressure, by means of a relatively heavy hydrocarbon material.

3. The herein described method of making 70 bricks, blocks, or the like, consisting in impregnating comminuted cypress wood with 65 a relatively light asphaltum residue of mineral oil, and then forming the impregnated material into solid form, under heavy pressure and by means of a relatively heavy asphaltum residue of mineral oil.

4. The herein described method of making 75 bricks, blocks, or the like, which consists in separating from each other the relatively light and heavy asphaltums constituting the residue of a mineral oil having an asphalt base, and from which oil the most volatile components have previously been extracted, soaking comminuted cypress wood in said lighter asphaltums to impregnate 80 the same therewith, mixing the impregnated comminuted wood with said heavier asphaltums, and uniting the whole under pressure into a solid mass, said heavier and lighter asphaltums recombining to form an approximately homogeneous compound 85 which entirely permeates the wood particles and acts as a binder therebetween.

In testimony whereof we affix our signatures.

JOSEPH WADE TUCKER.  
WILLIAM A. McCOOL.